

Patented July 14, 1942

2,290,018

# UNITED STATES PATENT OFFICE

2,290,018

## ALUMINUM ALLOY

Walter Bonsack, South Euclid, Ohio, assignor to  
The National Smelting Company, Cleveland,  
Ohio, a corporation of Ohio

No Drawing. Original application April 17, 1941,  
Serial No. 389,020. Divided and this applica-  
tion June 16, 1941, Serial No. 398,315

4 Claims. (Cl. 75—142)

This invention relates to alloys, and particularly to aluminum base alloys suitable for casting and working, and having high strength at ordinary and elevated temperatures.

This application is a division of my copending application Serial No. 389,020, filed April 17, 1941, for Aluminum alloys.

It is an object of this invention to produce alloys having relatively high elongation and relatively high tensile strength.

It is a further object of this invention to provide a relatively light alloy which may be easily cast and machined, which may be used at elevated temperatures without a rapid deterioration of desirable properties, and which may be readily treated with anodic treatment to give excellent lustre and finish.

It is a still further object of this invention to provide an alloy having a relatively high proportional limit and relatively high fatigue strength, and in which these properties may be obtained without heat treatment.

It has been found that an aluminum alloy containing iron, and having zinc and magnesium present in proper proportions, will produce an alloy that may be readily cast and have improved physical properties for use both at ordinary and elevated temperatures, and which may have these properties improved by heat treatment.

When magnesium and zinc are added to aluminum in the proper proportions, a ternary compound of aluminum, magnesium and zinc is formed, which compound is soluble in solid solution in the aluminum. The presence of this compound in relatively small amounts greatly improves the characteristics of aluminum and produces an alloy having high strength combined with high ductility, good casting and forging properties, good color, and excellent corrosion resistance. In calculating the amount of magnesium and zinc that should be present in the aluminum alloy to form the desired percentage of ternary compound, only magnesium which is not combined with silicon is to be calculated, as it is only such magnesium that is available to combine with zinc and aluminum to form the ternary compound.

The ternary compound is said by some investigators to have a composition having substantially the formula  $Al_3Mg_7Zn_3$ , and other investigators have considered the formula for the ternary compound as being  $Al_2Mg_3Zn_3$ . It will be seen that the amounts of magnesium and zinc relative to each other are quite similar in both formulas and, for the purposes of the improved alloy, the magnesium and zinc should be present in about the proportion necessary to form the ternary compound of either formula.

An excess of zinc, over and above that which cooperates with magnesium and aluminum to

form a ternary compound according to the above formula having the greatest proportion of zinc, increases the brittleness and decreases the ductility of the alloy. For this reason it is undesirable that zinc be present in quantities substantially greater than the amount to react to form such a ternary compound with magnesium and aluminum. The most desirable properties are obtained when the magnesium and the zinc are proportioned so that the ratio of magnesium (uncombined with any silicon) to zinc is about equal to the ratio represented by the formula  $Al_3Mg_7Zn_3$ , or somewhat larger as represented by the formula  $Al_2Mg_3Zn_3$ . A small amount of magnesium may be provided to replenish losses that may occur when the alloy metal is remelted.

Magnesium adds to the hardness and machining qualities of the alloy and, as above stated, should be present in an amount sufficient to combine with the zinc and aluminum present. In greater quantities magnesium tends to make the alloy sluggish, decreasing castability.

Magnesium and zinc have heretofore been added to aluminum in the proportion represented by the formula  $MgZn_2$ . It has been found, however, that a given percentage of ternary compound is more effective in producing desirable properties and, because the zinc content of the ternary alloys is less, they have a lower density.

The improved aluminum alloys may have the ternary compound of aluminum, zinc and magnesium present in an amount ranging from about 2% to 20%, the preferred range being between about 3% and 15%. At room temperature the ternary compound goes into solid solution in aluminum alloys in an amount of about 2%. The percentage in solid solution increases at high temperatures and decreases upon cooling, the excess precipitating out. Aluminum alloys containing the ternary compound may, therefore, be advantageously heat treated to improve their properties.

A small amount of silicon is usually present in aluminum alloys and from .15% to about .7% is desirable in alloys of the present invention which are to be forged or drawn; more than .7% is frequently desirable in casting alloys. Silicon combines with magnesium in preference to most elements, each part by weight of silicon combining with about 1.75%, by weight, of magnesium to form  $Mg_2Si$ . At least sufficient magnesium is therefore added to the alloy to combine with the silicon uncombined with any calcium to form  $Mg_2Si$ , and, in addition, to combine with all the zinc and form the ternary compound according to the formula  $Al_2Mg_3Zn_3$ .  $Mg_2Si$  is more stable than the ternary compound above mentioned and may be maintained in solid solution in aluminum alloys in an amount up to about 1.85%, which is the quantity of  $Mg_2Si$ .

present if the silicon is present in the alloy, and acts as a hardener, which is sometimes desirable in conjunction with the ternary compound. Mg<sub>2</sub>Si does not, however, make as efficient use of the magnesium as does the above mentioned ternary compound. Therefore, it is desirable to have the magnesium present on the rich side to prevent the silicon from being present in excess and taking magnesium away from the ternary compound.

If the alloy is desired particularly for casting purposes, more silicon, such as up to about 1.5%, may be present. If, however, a somewhat larger amount of silicon is present in the alloy than is desirable for the purpose for which the alloy is intended, and such amount of silicon is not too excessive, then a small amount of calcium may be added. Calcium has an even stronger affinity for silicon than has magnesium and, therefore, it can be used to reduce the amount of silicon available for combination with magnesium. The amount of the relatively expensive magnesium available for the formation of the ternary compound may thus be increased. Although much more than 1.85% silicide acts as a supplemental hardener and more than about 3% or so makes the alloy more sluggish and adversely affects the castability of the alloy, up to 3% is desirable, and more than 3% may, in some cases, be desirable in the production of hard castings having less intricate shapes, particularly when a large amount of the ternary compound is present in the alloy. Usually, however, the amount of silicon should be between .5% and 1.5%, especially in castings not heat treated. This is true even when calcium is present, although with the latter element more magnesium is available for formation of the ternary compound.

While 2% or 3% of the ternary compound of aluminum, magnesium and zinc improves the properties of aluminum or aluminum alloys having low silicon content, alloys containing such low percentages of a ternary compound are relatively difficult to cast.

An alloy containing 2% of the ternary compound may be used for casting purposes. The castability, however, is improved with an increase in the amount of ternary compound, and it is, therefore, preferred to have a larger percentage of the ternary compound present, such as 4% to 8%, for casting purposes. When the casting is more or less intricately shaped, still greater percentages, such as 10% to 15% or 20%, of the ternary compound may be present. For alloys to be forged or shaped after casting, the ternary compound should be present in the lower ranges, such as 2% to 8% or so, as the metal is less hard with the lower percentages of the ternary compound.

A larger proportion of the ternary compound and metals of the above hardening group may be present in alloys which are to be given a so-called "solution treatment" than in alloys to be given only an aging treatment, or those to be quenched from the casting mold and aged at relatively low temperatures. Thus, the desirable properties of the solution heat treated alloys may be obtained when they contain the ternary compound in amounts up to 20% or so, whereas less of the ternary compound, such as 4% to 15%, is preferred in alloys which are quenched upon removal from the mold and heat treated at a low temperature, or aged at room temperature.

It has generally been considered that aluminum alloys of magnesium containing iron much

above the impurity value in commercial aluminum are of little commercial value; but it has also now been found that an alloy containing the above described ternary compound, is improved by the presence of iron in suitable proportion.

Iron in suitable amounts further increases the hardness and tensile strength of the alloy without decreasing its ductility a substantial amount. A small amount of iron thus permits one to obtain

the properties desired with a smaller amount of magnesium and zinc. These alloys containing iron may be readily heat treated or age hardened to give somewhat superior properties, but the iron in combination with the ternary elements in the above proportion is also outstanding,

in that almost as desirable properties are obtained when castings are aged at room temperature without a heat treatment or quenching.

Iron has generally been considered to crystallize in large platelike crystals, which weaken the alloy. Iron in the presence of the ternary compound appears to crystallize in finely dispersed form, and the ternary compound also seems to be dispersed, thus producing a highly desirable alloy.

Iron in the amount of .4% or more in the alloys of the present invention gives noticeable effects in improving the properties of the alloy, and as much as 2% has been found to be desirable for

some purposes. For most castings it is desirable that the alloy have .6% or .7% to 1.5% of iron, although about 1% is usually preferred. The quantity of iron desired in the alloy depends also upon the quantity of other hardening ingredients

and upon the amount of ternary present, a given hardness and tensile strength often being obtainable with a relatively larger amount of iron and a relatively smaller amount of ternary compound, or a relatively smaller amount of iron and a relatively larger amount of ternary.

An aluminum base alloy containing .2% silicon and magnesium (uncombined with silicon) and zinc in the proportions represented by the formula Al<sub>3</sub>Mg<sub>2</sub>Zn<sub>3</sub>, and in sufficient amounts to produce 6% of this ternary compound in the alloy, was prepared. From this base alloy three different alloys were prepared by incorporating the proportions of iron indicated in the following Table 1, and chill cast in standard test bar molds. Several bars of each alloy were given the indicated heat treatments, that is, some of the bars of each alloy were removed from the mold while hot and allowed to cool in air, and then aged seven days at room temperature;

another set of bars was removed from the mold before the bars had cooled sufficiently to precipitate the hardening ingredients, then quenched in water and allowed to age at room temperature for seven days.

TABLE 1

| Alloy | Fe       | Elongation | Proportional limit    | Yield strength        | Tensile strength      | Brinell hardness     |
|-------|----------|------------|-----------------------|-----------------------|-----------------------|----------------------|
|       | Per cent | Per cent   | Lbs./in. <sup>2</sup> | Lbs./in. <sup>2</sup> | Lbs./in. <sup>2</sup> | kg./mm. <sup>2</sup> |
| 1*    | .81      | 6.2        | 16,100                | 23,300                | 36,900                | 79                   |
| 2*    | 1.34     | 4.4        | 19,200                | 26,400                | 39,500                | 85                   |
| 3*    | 1.87     | 5.4        | 18,500                | 25,300                | 39,600                | 84                   |
| 1**   | .81      | 7.9        | 16,400                | 23,100                | 39,400                | 79                   |
| 2**   | 1.34     | 5.0        | 19,400                | 26,600                | 41,100                | 85                   |
| 3**   | 1.87     | 5.8        | 17,400                | 25,000                | 40,400                | 83                   |

\*Alloy air-cooled; aged at room temperature seven days.

\*\*Alloy quenched; aged at room temperature seven days.

It is seen from the test results of the above table that, although the tensile strength may be

increased to some extent by a quenching treatment, almost equal results are obtained by simply air-cooling the casting and aging it at room temperature. Before the quenched casting is aged a tensile strength of over 30,000 lbs./sq. in. is obtained, while at the same time the casting has an elongation of 12%. In an aged casting a tensile strength of even greater than 40,000 lbs./sq. in., together with an elongation of almost 8%, is obtained. In an aged casting maximum elongation and substantially maximum strength are obtained when the iron content is about 1% or so.

When the quantity of ternary compound is increased, these maximum values may be obtained with a somewhat lower iron content, or higher maximum strength is obtained with the same iron content; the castability of the alloy may be also somewhat increased. It will be seen that, since the iron permits one to obtain exceptionally high elongation, combined with high tensile strength, without the necessity of even as much heat treatment as quenching from the mold, the alloy is especially useful for many purposes, such as large castings or forgings, wherein it is difficult to heat treat or quench.

Copper makes the alloy more responsive to heat treatment, and from 2% to about 1%, or even up to about 1.5%, copper may advantageously be present. Copper is a precipitation hardening ingredient, and the benefits of this element are obtainable when the alloy is subjected to heat treatment, which precipitates the copper from the solid solution. The presence of from .5% to 1.5% copper permits a reduction in the amount of ternary compound, which may be as low as 1%, and preferably should not exceed about 10% or 12%.

#### Example 1

An aluminum base alloy containing 6% of the above described ternary compound based on the formula  $Al_3Mg_7Zn_3$ , about 1% iron, about .3% silicon, and about .5% copper, was chill cast into test bars, quenched and aged seven days at room temperature. When tested, these test bars showed a tensile strength of about 41,200 lbs./sq. in., a yield strength of about 23,700 lbs./sq. in., a proportional limit of 17,400 lbs./sq. in., a hardness of about 81 Rockwell E, and an elongation of about 7.8%.

#### Example 2

When the aluminum base alloy of Example 1 contained only about .25% copper instead of .5% copper, the tensile strength was about 39,000 lbs./sq. in., and a yield strength of about 22,700 lbs./sq. in., a proportional limit of about 16,800 lbs./sq. in., a hardness of about 83 Rockwell E, and an elongation of about 7% were obtained.

Since the molecular proportion of zinc is never more than the molecular proportion of the relatively light magnesium in the ternary compound, it is seen that, in addition to high strength, the alloys are light in weight and are, therefore, especially adapted to aircraft construction and the like. This is particularly true when the quantity of ternary compound is sufficiently low so that the alloy may be drawn or rolled into structural members.

If the alloy contains uncombined silicon, about 1.75% magnesium is required to combine with each percent of uncombined silicon to form magnesium silicide ( $Mg_2Si$ ) before any ternary compound will be formed. For example, if 2% of the ternary compound on the basis of  $Al_3Mg_7Zn_3$  be

desired in an alloy having .3% silicon, the amount of magnesium to be added to form the ternary compound will be .45%, or about .5%, and the magnesium to combine with .3% silicon will be about .5%, making a total of about 1%.

The magnesium and zinc in an alloy containing .7% free silicon and 20%  $Al_3Mg_7Zn_3$  would be about 7% and 12%, respectively. The alloys described herein include aluminum, magnesium and zinc, the zinc being present in the amounts of 1.2% to 12% of the alloy, and the magnesium, uncombined with silicon, being proportioned to the zinc in the ranges of the formulas given for the ternary compound. The proportions for the formation of the ternary compound in the alloy exist when the magnesium is about 35% to 45% of the zinc content plus 175% of the silicon content. Most desirable properties may be obtained when the magnesium (uncombined with silicon) is in the lower portion of this range, or about 35% to 40% of the zinc.

In the above examples of alloys of the present invention it is to be noted that excellent tensile strength and hardness are obtainable in a relatively short time by aging at room temperature. A very astounding fact has been discovered, however, in connection with these alloys, namely, that the tensile strength may increase up to approximately 50% of its initial value by aging at room temperature for relatively long periods of time, such as a few months. The same improvement in tensile strength can, of course, be obtained relatively quickly by aging at temperatures above room temperature.

The improvement of properties is illustrated by the following table showing the improvement in an alloy containing a small percentage of silicon, about 6% ternary compound, about 1% iron, and about .2% titanium. The test bars were chill cast, quenched from the mold, and tested after aging at room temperature for the period indicated.

TABLE 2

| Aging time | Elongation | Tensile strength | Hardness   |
|------------|------------|------------------|------------|
|            |            |                  | Rockwell E |
| None       | 12         | 31,200           | 56         |
| 3 days     | 7.9        | 36,700           | 76         |
| 1 week     | 7.3        | 38,300           | 80         |
| 2 weeks    | 6.6        | 39,700           | 82         |
| 3 weeks    | 6.6        | 40,000           | 84         |
| 4 weeks    | 6.3        | 40,300           | 83         |
| 5 weeks    | 6.6        | 40,900           | 85         |
| 2 months   | 6.0        | 41,350           | 85.1       |
| 3 months   | 4.8        | 41,600           | 88.5       |
| 4 months   | 4.8        | 42,500           | 87.6       |
| 5 months   | 5.2        | 43,400           | 89.1       |
| 6 months   | 5.1        | 43,700           | 89.1       |

To obtain these exceptional properties in aluminum base alloys commonly in use one has to resort to a solution and aging heat treatment, whereas in alloys of the present invention it is not necessary to solution heat treat for improvement in properties.

The alloys of the present invention have good fatigue and tensile strength and a relatively high proportional limit, even at relatively high temperatures; they may be heat treated to improve and modify their properties; and they have sufficient ductility and hardness so that they can be used as sheets, rods, wire, structural shapes, castings, machine parts, etc. These alloys have a desirable color, high corrosion resistance, and may be anodically finished or highly polished with excellent results, and are suitable for many uses, among them being the production of cast-

ings which are shaped or formed to some extent after casting. The alloys having the lower percentages of ternary compound may even be forged at room temperature, and are thus useful for many special purposes.

It is to be understood that, in considering the amount of zinc and magnesium to add to aluminum alloys to form the ternary compound of aluminum, magnesium and zinc in the alloy, such magnesium as is necessary to combine with the uncombined silicon is not to be considered as part of the magnesium necessary to form the specified amount of ternary compound.

It is to be understood that the particular compounds disclosed and the procedure set forth are presented for purposes of explanation and illustration, and that various equivalents can be used and modifications of said procedure can be made without departing from my invention as defined in the appended claims.

What I claim is:

1. An aluminum base alloy containing magnesium, zinc, about .15% to 1.5% silicon, about .2% to 1.5% copper, and about .4% to 2% iron, with the balance substantially all aluminum and minor impurities, the percentage of zinc in the alloy being about 1.2% to 7.2%, and the amount of magnesium uncombined with the silicon being about 35% to about 45% of the zinc content, the total magnesium being within the range of about .5% to 7%.

2. An aluminum base alloy containing mag-

nesium, zinc, about .2% to 1.5% copper, silicon in an amount up to about 1.5%, and about .4% to 2% iron, with the balance substantially all aluminum and minor impurities, the percentage of zinc in the alloy being about .6% to 12%, and the amount of magnesium uncombined with the silicon being about 35% to about 45% of the zinc content, the total amount of magnesium being within the range of about .5% to 7%.

3. An aluminum base alloy containing magnesium, zinc, about .2% to 1.5% copper, silicon in an amount up to about 1.5%, and about .4% to 2% iron, with the balance substantially all aluminum and minor impurities, the percentage of zinc in the alloy being from about .6% up to about 6%, and the amount of magnesium uncombined with the silicon being about 35% to about 45% of the zinc content, the total amount of magnesium being within the range of about .5% to 6%.

4. An aluminum base alloy containing magnesium, zinc, about .2% to 1.5% copper, silicon in an amount up to about 1.5%, and about .4% to 2% iron, with the balance substantially all aluminum and minor impurities, the percentage of zinc in the alloy being from about .6% up to about 4.8%, and the amount of magnesium uncombined with the silicon being about 35% to about 45% of the zinc content, the total amount of magnesium being within the range of about .5% to 5%.

WALTER BONSACK.